

Patented Nov. 27, 1928.

1,692,856

# UNITED STATES PATENT OFFICE.

CLARENCE A. NASH, OF MILWAUKEE, WISCONSIN, ASSIGNOR TO THE CUTLER-HAMMER MFG. CO., OF MILWAUKEE, WISCONSIN, A CORPORATION OF WISCONSIN.

## PRODUCTION OF PLASTIC COMPOSITION MATERIALS.

No Drawing.

Application filed March 12, 1921. Serial No 451,806.

This invention relates to the production of plastic composition materials comprising or containing a phenolic condensation product binder and a relatively inert filler.

5 In the production of such materials it has heretofore been customary to effect an initial or incomplete reaction, in one or more stages, between a phenolic body and an active methylene substance under conditions such that 10 substantially half of such phenolic body is chemically combined with methylene substance and to effect impregnation of the filler with the incomplete condensation product so formed, the material being thereafter 15 molded and subjected to thorough heat treatment, either subsequent to or during the molding operation, for converting the material of the molded article to a hard and substantially infusible and insoluble state.

20 While the method just outlined is the outgrowth of protracted development and experimentation and results moreover in an exceedingly valuable product, certain difficulties thereof as well as certain deficiencies of 25 the product are recognized.

Thus difficulty has heretofore been experienced in producing uniformly an initial condensation product in the necessary or desired state of partial reaction, since such reaction tends, when once initiated, to progress with extreme rapidity such as to render control and arrest thereof at such desired stage exceedingly difficult.

Various expedients have been adopted for 35 the purpose of obviating such difficulty. Thus it has been proposed to effect initial reaction in the presence of only a reduced quantity of certain of the agents thereof, whereby the reaction must automatically 40 terminate at or near the desired point. Also in certain cases it has been proposed to effect repeated additions of quantities less than the total required quantity of certain agents, permitting each portion to react fully before 45 addition of the next. It has also been proposed to introduce various inert solvents for facilitating control and arrest of the reaction. Thus it has been proposed to utilize as the methylene body a water solution of 50 formaldehyde, the water then acting as a reaction retarding and controlling agent. However, in such cases it was found desirable or even necessary to stimulate the re-

action by a suitable condensing or catalytic agent and when such agent was employed in sufficient quantities to start the reaction the latter tended to progress with undue rapidity. Also the use of different oils, and similar solvents for retarding and controlling the reaction has been proposed.

A further and perhaps more serious difficulty of the aforementioned method relates to the character of the product formed thereby, which product has in the past proven not entirely satisfactory in certain physical respects, the cause of many of such deficiencies having been quite definitely ascertained as that of inadequate or incomplete impregnation of the filler material with the binder. Thus where a fibrous filler is employed under the conditions aforesaid the binder does not completely penetrate and saturate the individual fibres of the filler material but merely adheres as an exterior coating to such individual fibres whereby after the ordinary impregnating treatment and during certain disintegrating and other subsequent treatments the relatively hard resinous binder tends to become broken away from the strands or fibres and consequently the homogeneity of the material is greatly impaired.

An object of the present invention is that of effecting certain improvements in the aforescribed process and in the products thereof.

Another object is that of providing an improved process of the character stated enabling ready and accurate control of the progress of all stages of the reaction between the aforesaid agents, thereby permitting arrest of such reaction with accuracy and precision at any given or desired stage.

Another object is that of providing such a method enabling the rate of progress of the reaction to be varied at will within relatively wide limits whereby such reaction may be accelerated or may be retarded to practically any extent desired.

Another object is that of effecting a more thorough and complete impregnation of the 100 filler with the binder material to thereby effect a greater degree of homogeneity and improved physical properties of the product.

Another object is that of providing such a method enabling and facilitating formation 105 of products corresponding with practically

any desired stage of the reaction between the aforementioned agents as a result of a single continuous reaction; or optionally by the same reaction performed in any desired number of steps.

Other objects and advantages will herein after appear.

According to the present invention it is proposed to utilize the filler material itself

- 10 for rendering the progress of the aforementioned reaction amenable to control and to regulate the temperature of the agents undergoing reaction within certain fairly definite limits for effecting such control.
- 15 It has been found in practice both experimentally and commercially that the filler material, in proportions in which the same may satisfactorily be employed in the finished product, may be utilized as a highly efficient
- 20 agent for retardation of the progress of the reaction and that by maintaining suitable temperature control of the agents undergoing such reaction in the presence of the filler the rate of the reaction may be controlled
- 25 practically as desired.

Without limitation to any particular theory in accounting for the marked retarding effect of the filler material it is applicant's belief, which belief appears to be substantiated in practice, that the fillers ordinarily employed act as heat absorbing bodies whereby the heat liberated as a result of the reaction is dispersed or dissipated and hence the temperature of the agents tends to rise much less rapidly. Otherwise stated, the filler material may be regarded as having a diluting effect upon the various agents, whereby the molecules or molecular groups thereof are more or less separated and hence are less able to combine rapidly with one another.

- 30 Whether the effect be due to either of the aforementioned causes or to the same working in conjunction with one another or with other causes, it is known that if the heat employed
- 35 to start and promote the reaction be maintained below a fairly definite limit, which limit will ordinarily vary with the character of the filler material and of the active agents employed and with the proportion which the
- 40 quantity of such filler material bears to the quantity of such active agents, the rate of reaction may be maintained such that the reaction is self-arresting upon discontinuing the heat supplied; whereas if the quantity of
- 45 heat materially exceeds the aforementioned limit, the reaction tends to progress automatically and not to be so self-arresting.

It has been found that where binder constituents comprising cresol and hexamethylene tetramine in proportions to afford substantially or slightly more than one methylene group to each phenolic group present are caused to react in the presence of a comminuted fibrous asbestos filler in proportions of approximately 70% filler to 30% binder the re-

action is self-arresting as aforescribed if the supply of heat be so regulated that the temperature of the agents does not materially exceed 175° F. If the quantity of the filler be relatively decreased the reaction tends to 70 progress more rapidly at such temperature whereby such reaction may be more readily controlled if a lower temperature be maintained. However, constant stirring or other agitation of the agents tends to permit control at higher temperatures, whereby under suitable conditions the reaction may be adequately controlled although the temperature rise as high as 220° F., or even higher, whereas obviously at such temperature the total time 80 required to carry the reaction either to completion or to any given or desired intermediate stage is correspondingly reduced.

Thus under the aforementioned conditions of adequate temperature control it is entirely 85 feasible where the desired product corresponds with an incomplete reaction between the agents, by discontinuing or materially reducing the heat supply, to so far retard the progress of the reaction as to permit subject- 90 ion of samples of the product to the subsequent treatment which is desired or contemplated and to thereby determine the fitness of the product for such treatment.

By the foregoing steps it is thus possible to 95 effect direct formation of compounds containing all ingredients which are necessary or desirable in the finished product and at the exact stage of reaction at which the physical properties of the compound are best adapted to the 100 particular kind of subsequent treatment contemplated, the entire reaction being controllable with complete facility for arrest thereof with precision at the desired stage, whereas prior to development of the instant method 105 extreme difficulty has been experienced in effecting arrest of the reaction at an intermediate stage even approximating a given or desired stage thereof.

Also, if desired, the reaction when arrested 110 at a relatively early stage may be restarted at any time and again controlled as formerly for bringing the compound to the desired stage of reaction. In the interval between such successive treatments, the material may 115 be stored, transported or otherwise disposed of without detriment thereto.

Further, it is possible to prepare an initial 120 condensation product binder or resin by any of the heretofore known methods, such binder to contain the phenolic body and methylene substance in practically any desired proportion but preferably containing sufficient un- 125 combined phenolic body to combine with considerably more than half of the methylene body required in the completed product and to incorporate the filler in such binder. The compound so formed may be thereafter subjected to action of a controlled supply of heat 130 to restart the reaction either subsequent to or

during thorough mixing of the binder and filler, the latter then acting as before to retard the reaction and facilitate arrest thereof at the desired stage.

5 Such incorporation of the filler in the binder prior to reaction of the constituents of the latter, or at a relatively early stage of such reaction, the binder being then in a relatively softer and more fluid state than at later 10 stages of the reaction, facilitates and promotes a much more thorough and complete impregnation of the individual portions, particles or fibres of the filler with binder substance than can be obtained after such later 15 stages of the reaction have been reached. Such more thorough impregnation of the filler with the binder in turn serves to effect very marked improvements in physical properties of the finished product particularly 20 where the subsequent treatment involves forming or molding steps, which steps moreover are facilitated by the resultant increased homogeneity of the compound.

As exemplary of the foregoing method, the 25 following preferred procedure may be described: 50 pounds of asbestos is placed in a kneading machine or other suitable form mixer, together with 16.75 pounds of cresol in which 3.3 pounds of hexamethylenetetra- 30 ramine has been dissolved. Such ingredients are mixed with one another for from twenty to thirty minutes, or until a homogeneous mass is effected, whereof the asbestos filler is thoroughly impregnated with the cresol of the 35 binder. Subsequently to such mixing operation the compound is placed in a drier and subjected to a moderate degree of heat for initiating chemical reaction between the cresol and hexamethylenetetramine, the mass undergoing reaction being stirred, rotated or otherwise agitated to prevent unequal or local heating, and the supply of heat being so controlled that the temperature of the mass does not materially exceed 175° F. The heating 40 is continued until the desired incomplete stage of the reaction is reached, the supply of heat being then discontinued whereupon the reaction ceases.

The compound containing all the essential ingredients of the finished article is thus brought by a single simple and readily controlled reaction to a chemical condition suitable for molding or other subsequent treatment. However, prior to such treatment the 45 material is ordinarily subjected to certain known treatments which may include cooling, disintegrating, screening and others.

In commercial practice it is desirable to 50 carry out the foregoing treatment of the material in a closed vessel with constant agitation to prevent local heating, suitable means being provided for permitting escape of the liberated ammonia when the internal pressure reaches a given value, and for collecting the ammonia so escaping. Good results are

also attainable by treating in a closed oven without special provision for keeping constant the relative amounts of the agents.

It is also possible to effect the reaction without agitation of the material if the same be 70 treated while spread in the form of thin layers or sheets and preferably subjected on all sides to like temperature conditions.

If the product of the foregoing step is intended for subjection to a quick molding operation at ordinary temperatures the foregoing reaction is preferably arrested at a stage such that substantially half the cresol remains chemically uncombined with hexamethylenetetramine whereas if hot molding 80 of the product is contemplated the reaction may be permitted to progress considerably farther.

To facilitate arrest of the reaction the supply of heat should be so regulated that the 85 temperature of the compound undergoing reaction does not materially exceed 175 degrees F., and under such conditions of heat control, the reaction is self arresting upon simple discontinuance of the heat supply. By regulating the temperature between the aforementioned upper limit and a lower limit corresponding with the lowest temperature at which chemical combination of the aforementioned substances is sustained, the rate of reaction may be so controlled that the time required to convert the uncombined agents to a state suitable for cold molding may be varied from approximately eight hours to fifteen hours or even longer, and at any time during such period the reaction may be terminated by simply cutting off the heat.

For producing a hot molding compound the heat treatment may be continued for a much longer period as from seventy-five to 100 one hundred hours, the time being in either case somewhat dependent upon the character of the filler employed and upon the nature and physical properties required in the finished article.

The degree of progress of the reaction may be ascertained at any time by any of the tests heretofore known and employed, whereas obviously if desired the supply of heat may be reduced or temporarily discontinued at any time and a sample of the product submitted to molding or other subsequent treatment under conditions similar to those contemplated, in order to ascertain the fitness of the product for such subsequent treatment.

If the product of such reaction is not intended for immediate subjection to the succeeding steps of molding and the like it is preferable to discontinue the reaction at a relatively early stage as when substantially two-thirds of the cresol remains chemically uncombined with methylene. The product in this condition may be stored for an indefinite period of time without deterioration or may be transported or otherwise handled, a brief 120

additional heat treatment under the conditions described being thereafter sufficient to render the product suitable for the molding or other subsequent treatment desired.

- 5 As a substitute for the foregoing steps, or certain thereof, it is possible and in certain instances desirable to mix the filler with a partially reacted condensation product, for example, one in which approximately but one-  
10 third of the total quantity of cresol required is combined with methylene substance, the aforementioned agents being present in substantially the proportions in which the same are adapted to effect complete combination  
15 with one another, and to subject the mix to a heat treatment similar to that described for bringing the compound to the desired state of reaction. Also it is possible to employ a phenolic condensation product wherein sub-  
20 stantially half the phenolic body is combined with methylene and to incorporate therewith, prior to or concurrently with the addition of the filler, a quantity of unreacted cresol or the like sufficient to pro-  
25 vide the desired softness and fluidity of the binder, a corresponding amount of methylene substance being also incorporated, either at the same time or subsequently, to maintain a suitable proportionality of the  
30 agents.

A typical mix suitable for performance of the latter-mentioned steps may be composed as follows:—11 pounds of phenolic condensation resin comprising about 10 phenolic  
35 groups to six methylene groups; cresol 6 pounds; hexamethylenetetramine (dissolved in the cresol) 2.4 pounds; asbestos 50 pounds.

In each of the foregoing examples the mixing operation may be promoted and a more thorough impregnation of the filler secured if the latter, prior to mixing with the binder, be moistened with a small quantity of a suitable solvent. Thus from one-half to one pint of coal tar oil may be preliminarily added to  
45 and mixed with the aforementioned quantity of the asbestos filler. Optionally such solvent may be added to the binder ingredients rather than to the filler, or small quantities of paraffin, fats, waxes or gums, up to one percent  
50 by weight of the binder may be added to the binder or mixed with the filler.

In each of the aforescribed methods it is to be understood that substances other than those specifically mentioned may be substituted therefor. Thus the cresol may be replaced by phenol or a homologue thereof whereas the hexamethylenetetramine or formaldehyde may be similarly replaced by a polymer thereof or by any other active methylene substance suitable for the purpose. Also the filler may comprise comminuted asbestos, wood fibre, mica flock, infusorial earth or mixtures of any of the foregoing or other substances regularly employed for such purposes.

What I claim as new and desire to secure by Letters Patent is:

1. A process of producing plastic composition material having as constituents a condensation product binder produced from a phenolic body and an active methylene containing substance, and a relatively inert filler, which comprises the step of effecting reaction of the complete ingredients of the binder after mixture thereof with the filler and prior to molding of the mixture, such filler being added in such quantities as to enable arrest of such reaction at a given stage thereof.

2. A process of producing plastic composition material having as constituents a condensation product binder produced from a phenolic body and an active methylene containing substance substantially in the absence of water, and a relatively inert filler, which is characterized by early incorporation in the complete binder constituents of sufficient filler material to facilitate control of progress of the condensation reaction through temperature control of the reaction mixture, such reaction being effected prior to molding of the material.

3. A process of producing plastic composition material whose constituents include a filler which is relatively inert chemically under the conditions imposed and a binder including products of an incomplete chemical reaction of a phenolic body and an active methylene containing substance which reaction tends to progress at an abnormal rate, which comprises effecting reaction of the complete ingredients of the binder in the presence of sufficient filler material to facilitate control of progress of the reaction by temperature control of the reaction mixture, such reaction being effected prior to molding of the material.

4. The process of producing plastic composition material having as constituents a relatively inert filler and a binder including a phenolic body and an active methylene containing substance, which ingredients are potentially reactive for producing a substantially anhydrous condensation product, which comprises effecting chemical reaction involving the complete constituents of the binder in the presence of a sufficient quantity of the filler to facilitate control of reaction progress through controlling the temperature of the reacting agents, such reaction being effected prior to molding of the materials.

5. The process of producing plastic composition material including as constituents a relatively inert filler and a binder having constituents, comprising a phenolic body and an active methylene containing substance, which are potentially reactive to produce a substantially anhydrous condensation product, which comprises mixing a quantity of the filler with a body including potentially

- reactive complete constituents of the binder, heating the mixture to a temperature above the reaction temperature of such binder constituents for promoting reaction thereof and 5 adjusting such quantity of the filler to facilitate arrest of the reaction through controlling the temperature of such constituents, such reaction being effected prior to molding of the material.
- 10 6. The process of producing plastic composition material including as constituents a relatively inert filler and a binder having ingredients, comprising a phenolic body and an active methylene containing substance, 15 which are potentially reactive for producing a substantially anhydrous condensation product, which comprises mixing with a body including potentially reactive complete ingredients of the binder a quantity of the filler material sufficient to render the reaction amenable to temperature control, heating the mixture to a temperature above the reaction temperature but below the temperature at 20 which the reaction is self maintaining under such condition, utilizing such filler material to control the progress of the resultant reaction and discontinuing the supply of heat for arrest of the reaction as desired, such reaction being effected prior to molding of the 25 material.
- 30 7. The process of producing plastic composition material, which comprises mixing together a substantially inert filler and binder ingredients comprising phenolic and methylene substances in substantially the proportions in which said substances are adapted to effect complete chemical combination with one another by a reaction which tends to resist arrest thereof, at least considerably more than half the total quantity of such 40 substances present being in a potentially reactive state and the filler being present in sufficient quantities to render the reaction amenable to temperature control, 45 heat treating the mixture below the temperature at which the resultant reaction becomes automatic and utilizing the filler in controlling arrest of such reaction as desired, such reaction being effected prior to molding 50 of the material.
- 55 8. The process of producing plastic composition material which comprises mixing together a substantially inert filler and binder comprising phenolic and substantially anhydrous methylene substances in proportions providing for substantially complete chemical combination thereof, at least considerably more than fifty percent of the total quantity of such substances present being in a potentially reactive state, and the filler being present in sufficient quantities to render the reaction amenable to temperature control, heat treating the mixture below the temperature at which the resultant reaction becomes automatic, utilizing the filler in controlling such 60 reaction and discontinuing such heat treatment for arrest of the reaction.
- 65 9. The process which comprises mixing together phenolic condensation product constituents in proportions to provide in such product substantially thirteen methylene groups to each twelve phenolic groups, at least considerably more than half the total number of the respective groups of such constituents being in a state rendering the same capable of effecting chemical combination with one another, incorporating in such mixture a relatively inert filler, subjecting the compound to prolonged heat treatment at 70 moderate temperature above that at which the potentially reactive agents are adapted to combine, discontinuing the heat treatment for arrest of the resultant reaction at a stage such that substantially half the total number of the respective groups present are chemically combined with one another and thereafter subjecting the product to a further heat treatment for carrying forward the reaction. 75
- 80 10. The process which comprises mixing together cresol and hexamethylenetetramine in proportions affording approximately six molecules of the former to one molecule of the latter, incorporating in the mixture a quantity of a substantially inert filler material, heat treating the resultant compound for 85 several hours at a temperature of approximately 175 degrees F., interrupting the supply of heat for arrest of the resultant reaction at a stage wherein approximately half the phenolic groups present are chemically combined with methylene groups and renewing the heat treatment for advancing the reaction to a stage wherein the product is in a condition suitable for subsequent treatment. 90
- 95 11. The process of producing articles comprising or containing a substantially anhydrous condensation product binder of a phenolic body and an active methylene containing substance, and a relatively inert filler, which comprises effecting a reaction involving chemically active complete constituents of the product after addition of sufficient filler material thereto to enable control and arrest of the reaction through temperature control of the reaction mixture, arresting the reaction 100 at a given incomplete stage thereof through such temperature control prior to molding, and then subjecting the resultant compound to subsequent treatment including thorough heat treatment for curing. 105
- 115 12. The process of producing articles comprising or containing a substantially anhydrous condensation product of a phenolic body and an active methylene containing substance, and a relatively inert filler, which comprises effecting a reaction involving chemically active complete constituents of the product after addition of sufficient filler material thereto to enable control and arrest of the reaction through temperature control of the 120 125 130 reaction.

- reaction mixture, arresting the reaction at a given incomplete stage through such temperature control, and thereafter subjecting the resultant compound to treatment including forming and heat treating to complete the reaction.
13. The process of producing articles comprising or containing a substantially anhydrous condensation product of a phenolic body and an active methylene containing substance, and a relatively inert filler, which comprises effecting a reaction involving chemically active complete constituents of the product after addition of sufficient filler material thereto to retard progress of such reaction, effecting temperature control for arresting the reaction at a given incomplete stage thereof prior to molding of the compound and subjecting the resultant compound to subsequent treatment including molding under pressure and heat treatment to complete the reaction.
14. The process of producing plastic composition material adapted to form giving treatment and heat hardening, which comprises effecting partial condensation reaction between the required total quantities of substances capable of furnishing approximately equal numbers of phenolic and methylene groups respectively, such partial condensation reaction being effected prior to molding of the material and being maintained amenable to control by incorporating with the potentially reactive substances a quantity of non-reactive material sufficient to retard said reaction, said non-reactive material being adapted to remain in situ as a constituent of the product.
15. In a process of producing plastic material by an incomplete condensation reaction of a phenolic body and an active methylene containing substance, which reaction tends to approach completion prematurely, the step which comprises retarding such reaction by causing at least certain stages thereof to be enacted prior to molding in the presence of a reaction retarding quantity of a material adapted to remain in situ as a constituent of the product.
16. In a process of producing plastic material comprising a relatively inert filler and a binder which is the product of incomplete condensation of the total quantities of phenolic and methylene substances employed by a reaction which tends to approach comple-
- tion prematurely, the step which comprises effecting at least certain stages of such incomplete condensation after incorporation of the filler and prior to molding of the material, to provide for retardation of the later stages of such incomplete condensation.
17. The process of producing plastic material comprising a relatively inert filler and a binder which is the product of incomplete condensation of phenolic and methylene substances by a reaction which tends to approach completion prematurely, which comprises incorporation of the filler with the complete ingredients of the binder at a stage such as to provide for retardation of the later stages of the incomplete condensation reaction prior to molding, as a result of the presence of the filler, and supplementary temperature control of the reacting ingredients for control and arrest of the reaction to render said material adaptable for molding under pressure.
18. A composition material comprising a relatively inert filler and a binder having approximately equal numbers of phenolic and methylene groups, at least substantially more than half of the phenolic groups being uncombined with methylene groups and being free, and which except for the presence of said filler would unite with one another by a reaction which when initiated tends to proceed to completion prematurely.
19. A plastic composition material suitable for molding, which comprises a phenolic body and an active methylene containing substance reacted prior to molding of the material in the presence of a quantity of filler sufficient to render such reaction amenable to quantitative control through heat regulation.
20. A plastic composition material suitable for molding, which comprises complete condensation product constituents including a phenolic body and an active methylene containing substance reacted together in the presence of a quantity of filler to a stage wherein substantially one-half of the phenolic groups present are in a potentially reactive state, the quantity of filler employed being so proportioned with reference to the quantity of condensation product constituents as to render the reaction amenable to control and arrest at the stage aforementioned through temperature regulation.

In witness whereof, I have hereunto subscribed my name.

CLARENCE A. NASH.